

Patented June 18, 1929.

1,717,798

# UNITED STATES PATENT OFFICE.

ROBERT A. MARR, OF NORFOLK, VIRGINIA.

## PROCESS OF MAKING PULP.

No Drawing. Application filed March 27, 1924, Serial No. 702,442. Renewed March 15, 1929.

- The present invention relates to the production of pulp and pulp products from wood and other cellulosic and ligneous material, and the process is applicable to all kinds of wood, including woods that are hard, soft, porous, non-porous, also other equivalent materials, e. g. cane, bamboo, straw, sedges and other marsh growth, banana stalks, cocoanut husks and the like.
- 10 The process consists essentially in first boiling the wood in a solution containing sodium nitrate or other nitrate of an alkali-forming metal, such as potassium nitrate, calcium nitrate, magnesium nitrate, although other nitrates can be employed, and it is not by intention to restrict the present case to the use of a particular nitrate or a group of such nitrates. However, the nitrates of the alkali-forming metals are generally cheaper and somewhat more satisfactory than any other nitrate with which I have experimented. After the material has been in the solution of nitrate, the same is removed from the solution, is preferably soaked for a time in cold water, after which it is run through pressure rolls or otherwise crushed and is then run through a pulper, with water, and is then preferably run into a beater in which it is beaten, preferably with the roll raised a substantial distance above the bed-plate, (3 to 5 turns) after which it may be sheeted or a portion of the cementitious matter may first be removed from the pulped material, either before, during or after the beating operation, before being converted into sheets. The pulp can be produced converted into sheets in the form of paper or card-board, or it can be converted into other shaped articles, in a manner well understood in the art.
- 30 40 The following examples are given, but it is to be understood that they are given merely for the purpose of illustration and not as restricting the invention thereto.
- Example 1.*—Blocks of spruce in a dried condition, chips of spruce containing about say 40% of water, and blocks of yellow poplar were introduced into a digester such as is used in making pulp by the well known processes, including the soda process, sulphite process and the like, sufficient of the solution being used to completely cover the woody material. The mass was then heated until a pressure of about 110 lbs., existed in the digester, which condition was continued for about an hour, after which the solution was allowed to cool more or less and the material removed from the digester. The total time that the pressure was above 80 lbs. in the digester was considered as the effective cooking period, this amounting to two hours.
- 50 60 The treated material was then removed from the digester liquor, was placed in a tank of cold water, for several hours and the materials were then run through crushing rollers, then with water through a pulper, and into a beater. The beating was commenced with the roll of the beater raised about six turns above the bed, and the roll was gradually lowered to about 3 turns of the bed. The beating was continued for half an hour, after which a portion of the pulp was sheeted and dried without washing. Another portion of the pulp was first washed, being given a light washing, with a spray of water, and was then sheeted. Another portion was further beaten for half an hour and sheeted. Another portion was further beaten for half an hour, at about the end of the beating operation, size and alum were added in the amounts commonly used in sizing paper. In other instances portions of the pulp were washed and then sized, and then sheeted.
- 70 80 90 100 110 *Example 2.*—Blocks of spruce wood, in a substantially air dry state were placed in the liquor remaining from the above treatment, and heat applied. About three-quarters of an hour were necessary before the pressure reached one hundred pounds and the pressure was maintained at one hundred pounds for about an hour, after which the liquor was allowed to cool somewhat and the blocks removed from the digester and placed in cold water overnight. The following day these were worked up as above indicated.
- Example 3.*—Blocks of air dry spruce wood, spruce wood in the form of chips containing about 40% of moisture, yellow poplar and green cane were placed in the solution remaining from the above experiment and were cooked in the manner above indicated. The solution was heated up in this experiment until a pressure of 110 lbs. existed in the digester, which condition was maintained for two hours and twenty minutes, the heat then cut off and the material allowed to cool, after which it was removed from the liquor and treated in the manner above referred to. I call attention to the fact that the same solution was used over for the three cooks above referred to, and

my experiments indicate that the solution can be used a very great number of times before the same becomes sufficiently impure to make it necessary to discard the same.

- 5 The heating of the solution, by blowing in steam, will of course dilute the solution to a certain extent, and it is accordingly advisable after each fourth or fifth cook, to add a little more nitrate, in order to bring 10 the strength back to that originally employed.

The sheeted products resulting from the treatment of spruce wood were of a light buff color. All of the sheeted material produced in the above experiments was found to be very strong, similar to kraft paper of the best grade. The product produced from poplar wood was of a substantially darker color than that produced from spruce, being 20 a medium brown. This product was particularly strong and tough and was adapted for very strong wrapping paper.

During the cooking operation, the liquor acquires a yellowish color and is found to 25 have a pronounced caramel odor.

My experiments indicate that something over 95% of the dry matter of the wood can be recovered in the form of unwashed pulp, but it is to be understood that any desired proportion of the cementitious matter can be washed out after the pulping operation, either before, during or after the beating operation. The cementitious matter thus washed out can be recovered and can 35 be used in making various plastic shaped articles.

The use of nitrates seems in some respects to be somewhat better than sulfates as referred to in some of my copending applications, and also seems to be somewhat better than sodium chloride referred to in another copending application of mine. From the same wood, the pulp product produced when nitrate forms the digestive solution, seems to 40 be somewhat tougher and stronger than the solution used in sodium chloride.

The pulp produced can be used not only for making paper and other similar products, but for making card-board and various 50 molded articles.

While I have above referred to the use of a solution of 1.6%, it is to be understood that solutions of other strengths can be employed, for instance, solutions of 1 to 4%. In some 55 instances this range can be somewhat exceeded, but solutions of below 1% strength require substantially longer periods and solutions of considerably over 4% strength are likely in some cases to somewhat injure 60 the product.

It will be observed that while in many of the pulp-making processes heretofore used in this country, it has been customary to boil the wood or other material under high pressure until the same has been converted into 65

a pulp, and the cementitious matter has been entirely destroyed, in the process of the present application I preferably boil only until the cementitious matter has been converted into a readily friable condition so 70 that the material can be readily crushed by being run between heavy rollers, or by being treated in an edge runner mill or similar device.

I call attention to the fact that while in 75 the processes heretofore generally used in this country highly concentrated solutions of the chemicals are employed, I use in the present case preferably a dilute solution, such as a solution of 1.6% as given in the 80 above examples, although various strengths between about 1% and about 4% can be employed. The pressure during the cooking operation does not have to exceed about 80 to 100 lbs., or 120 lbs., per square inch, 85 and the cooking operation is relatively short, as compared with the cooking operation in the prior processes, commonly in use in this country, such as the sulfite process, the soda process and the sodium sulfide process (so 90 called sulfate process).

I claim:

1. A process which comprises boiling cel- 95 lulose and ligneous material with a dilute aqueous solution of a soluble nitrate, soaking in water and mechanically reducing to a pulp.

2. A process which comprises boiling cel- 100 lulose and ligneous material with a solution of a nitrate of an alkali-forming metal of substantially below 4% concentration, and continuing the treatment until the cementitious matter is converted into a readily friable condition but not until the material has been converted into a pulpy mass, there- 105 after soaking in water and mechanically reducing to a pulp.

3. A process which comprises boiling cel- 110 lulose and ligneous material with a solution of sodium nitrate, and continuing the treat- ment until the cementitious matter is con- 115 verted into a readily friable condition but not until the material has been converted into a pulpy mass, thereafter soaking in water and mechanically reducing to a pulp. 115

4. A process which comprises boiling cel- 120 lulose and ligneous material with a solution of sodium nitrate of about 1 to 4% strength, and continuing the treatment until the cementitious matter is converted into a readily friable condition but not until the material has been converted into a pulpy mass, thereafter soaking in water and mechanically reducing to a pulp. 120

5. A process which comprises boiling cel- 125 lulose and ligneous material with a 1 to 2% solution of a nitrate of an alkali-forming metal, and continuing the treatment until the cementitious matter is converted into a readily friable condition but not un- 130

til the material has been converted into a pulpy mass, thereafter soaking in water and mechanically reducing to a pulp.

6. A process which comprises boiling cellulose and ligneous material with a 1 to 2% solution of a nitrate of an alkali-forming metal, and continuing the treatment until the cementitious matter is converted into a readily friable condition but not until the

material has been converted into a pulpy mass, thereafter crushing the cooked material and mechanically pulping the same without subjecting the same to the usual grinding operation used in making wood pulp.

15

In testimony whereof I affix my signature.

ROBERT A. MARR.